

Jan. 10, 1939.

A. P. ANDERSON

2,143,531

PROCESS FOR REFINING MINERAL OILS

Filed March 27, 1936



Inventor: Alvin P. Anderson

By his Attorney: D. A. Anderson

## UNITED STATES PATENT OFFICE

2,143,531

## PROCESS FOR REFINING MINERAL OILS

Alvin P. Anderson, Alton, Ill., assignor to Shell Development Company, San Francisco, Calif., a corporation of Delaware

Application March 27, 1936, Serial No. 71,197

11 Claims. (Cl. 196—13)

This invention relates to the refining of mineral lubricating oils, and is particularly concerned with a process for the acid treatment of highly paraffinic oils which it is difficult to refine by the known sulfuric acid treating methods.

Mineral oils used for lubrication are often subjected to treatment with sulfuric acid during processing to decrease their tendencies to discolor and to form sludge and other undesirable products. These undesirable, unstable components are normally present but are removed by the acid. Different methods of applying the acid to the stock treated have been developed to obtain economies or operating advantages. The most common methods are the direct mixing under optimum conditions in batch agitators or continuous mixers and settling the resulting sludge in the agitator or in separate settlers, and to mix the acid with suitable mechanical mixers and then to remove the sludge by centrifuging.

There are oils, however, that contain these unstable materials but which cannot be acid treated by the normal procedures because the sludge particles are too finely dispersed forming so-called pepper sludge which cannot be removed by ordinary means. These oils are highly paraffinic in nature and comprise oils distilled from certain Pennsylvanian crudes and oils produced by selective extraction with solvents in such a way that the paraffinic portion (raffinate) which is to be finished to produce lubricating oils has a viscosity index (Dean and Davis) higher than about 70 or 80. The viscosity index is a measure of paraffinicity and is described in Chemical and Metallurgical Engineering 1929, vol. 36, No. 10, page 618 (Viscosity Variations of Oils with Temperature, by E. W. Dean and G. H. B. Davis). Highly paraffinic oils such as Pennsylvanian may have viscosity indices of approximately one hundred, while naphthenic oils may have zero or negative viscosity indices.

The practice with such oils is to treat with clay alone in sufficient quantities to obtain the desired color, etc. As far as I know, no generally satisfactory method of acid treating such oils with sulfuric acid has been revealed. It is known that very small amounts of acid, two to three pounds per barrel, or that very large amounts of acid, fifty to sixty pounds per barrel, can be applied successfully. These amounts are either too small to effect any appreciable savings in clay or too large to be economical except for certain high priced oils for special purposes.

The object of this invention is to provide a simple but effective means of acid treating paraf-

finic stocks with any amount of acid desired to effect savings in clay and to increase the stability of the finished oil. In accordance with the present invention it has been found that small quantities of the extract (naphthenic portion from solvent extraction) and unsaturated asphaltic materials are very effective as coagulating agents and that with their aid paraffinic oils can be readily acid treated by otherwise normal methods. These materials can be employed separately or together.

My invention may be further understood by referring to the accompanying drawing, which is a schematic flow diagram illustrating one embodiment of my invention.

In the drawing, 1 and 2 are mixing and agitating devices; 3 is a settling tank adapted for the separation of immiscible liquids; 4 is an extraction apparatus, which may be a series of mixers and settlers, or a contact tower provided with means for the countercurrent flow of liquids; 5 and 6 are continuous settlers, adapted to separate acid sludge from oil; 7, 8, 9 and 10 are separating apparatus, such as combinations of evaporating and distilling units; 11 is an apparatus for clay treatment; 12 and 13 are condensers; and 14, 15 and 16 are storage tanks for a selective solvent, naphtha, and sulfuric acid, respectively; all interconnected as shown as hereafter described, and provided with pumps, flow control devices, heat exchangers, and other auxiliary equipment, not shown.

My process will first be described as applied to the treatment of an oil containing a sufficient quantity of hydrocarbons of low viscosity indices to necessitate its extraction with selective solvent to improve its temperature-viscosity characteristics. In this type of process, the initial mineral oil fraction is introduced into the extraction apparatus 4 through a conduit 17 and valve 18, and extracted therein with a selective solvent for aromatic or naphthenic oils, such as liquid sulfur dioxide, furfural,  $\beta\beta'$  dichloroethyl ether, cresol, phenol, nitrobenzene or any other equivalent selective solvent or mixture of solvents such as a mixture of sulfur dioxide and benzol or kerosene extract supplied from the tank 14 through a valve 19. The liquid raffinate and extract phases produced in the extraction apparatus are withdrawn at 20 and 21, respectively, and treated in the apparatus 8 and 9 to recover the selective solvent, which is condensed and returned to the tank 14. The extracted raffinate oil is withdrawn at 22 and the extract at 23.

The raffinate oil is next flown through a valve 55

24 and intimately mixed with a proper quantity of concentrated sulfuric acid in the mixer 2. The concentration of the acid may be varied to suit the viscosity of the oil, and may, for example, be 5 between 85 and 100% and will generally be higher than 90% for the more viscous oils. Moreover, it may often be desirable to employ fuming sulfuric acid, as for example, 20% oleum, particularly in the refining of viscous white oils. The 10 quantity of acid will also vary with the stock being treated, and may, for example, be between five to fifty pounds of 66° Bé. acid per barrel (42 U. S. gals.). The temperature of the agitation may, for example, be between 10° C. and 60° C., 15 but my process is not restricted to these limits.

The contacting of the acid and oil in the mixer 2 may be effected with air; or the mixer 2 may be provided with a propeller and draft tube. After the acid has acted on the impurities in the oil, the mixture of oil, acid and sludge is fed 20 through a conduit 25 to the settler 5, the sour oil overflowing the conical settling chamber into the peripheral launder 26, and being withdrawn through valves 27 and 28 for further treatment, 25 such as dewaxing or neutralization with soda or clay treatment. If clay treatment is to be employed the sour oil is introduced into the apparatus 11 where it is contacted with clay, preferably at an elevated temperature above about 30 140° C., but below cracking temperature, the finished oil being withdrawn at 29.

The acid sludge is continuously pumped from the bottom of the conical settler 5 and discharged at 30.

35 The acid treatment can in many cases be carried out more readily by diluting the oil with a light distillate, such as propane, gasoline, naphtha or a similar hydrocarbon distillate. This is particularly desirable when it is desired to dewax 40 the oil in its diluted state following the acid treatment. For this purpose, the diluent may be supplied from the tank 15 through a valve 31. If desired, the diluent may be recovered from the sour oil prior to clay treatment by means of the 45 apparatus 10. A further economy from the use of the diluent arises from the possibility of improving the yield by washing the acid sludge to recover entrained oil. This may be effected by feeding the acid sludge and the diluent through 50 valves 32 and 33 into a mixer 34, and separating the resulting mixture in the settler 6, the diluent with dissolved oil being recycled through the valve 35 and the sludge withdrawn at 36.

55 It is moreover, in many cases desirable to acid treat the raffinate oil in the presence of dissolved selective solvent, such as sulfur dioxide. In this case, the separating apparatus 8 may be eliminated, and the raffinate phase from the extraction apparatus 4 fed into the mixer through by-pass valve 37.

60 As was pointed out above, when the raffinate oil which is treated with acid has a viscosity index greater than about 70 or 80, it is often difficult to remove the sludge from the oil in the settler 5. 65 In accordance with the present invention, I overcome this difficulty by introducing a small amount of the aromatic extract into the oil. This extract is herein designated as "SO<sub>2</sub> soluble", although it may be obtained with the aid of any 70 similar selective solvent. Between 1 and 10% of this extract based on the weight of oil to be acid treated are generally sufficient, altho I am not restricted to this exact range.

75 To introduce the SO<sub>2</sub> soluble extract, I may open the valve 38, so as to cause a portion of the

extract oil to flow through the conduit 39 into the mixer 2. It should be noted that the amount of extract thus introduced is not sufficient to impair the viscosity index of the final product to any marked degree; nor is the addition of this 5 extract equivalent to operating the extraction apparatus 4 in a manner to remove a smaller quantity of extract, because the components of the oil which are particularly effective in improving the separation of the acid sludge in the settler 10 5 are those which are the most soluble in selective solvents, and would for this reason be removed from the oil altho a smaller amount of selective solvent were employed in the extraction.

It is also possible to concentrate the most 15 soluble components of the oil by subjecting the extract flowing through the conduit 21 to a treatment for the separation of the less soluble hydrocarbons. Thus, the initial extract in the conduit 21 may be chilled to cause the formation of two 20 secondary liquid phases, the hydrocarbons which remain dissolved in the selective solvent, or a portion of them fed through the conduit 39; or a portion of the selective solvent may be separated 25 by distillation, and the resulting solvent-poor extract phase chilled to cause a similar separation into secondary liquid phases.

According to an alternative method of concentrating the most soluble components of the oil, all or a portion of the initial oil may be fed to 30 the mixer 1 through a valve 40 and mixed with selective solvent, fed through a valve 41. The resulting mixture is transferred to the settling tank 3, where the mixture is permitted to stratify, the oil phase being removed through the conduit 35 42, and the extract being withdrawn at 43 and treated in the apparatus 7 to recover the selective solvent. The quantity of the solvent supplied through the valve 41 is preferably small, and the temperature is such that only a small amount of 40 the extract phase is formed, the greater part of the oil being thereby withdrawn as the oil phase. In this manner only the most soluble components are dissolved in the extract phase, and the operation of the apparatus 4 is not adversely affected, 45 since only sufficient oil is preferably passed through the valve 40 to provide the desired quantity of SO<sub>2</sub> soluble extract for admixture with the oil to be acid treated, the bulk of the oil being fed into the apparatus 4 through the valve 18. 50 The SO<sub>2</sub> soluble extract from the apparatus 7 is introduced into the mixer 2 through conduits 44 and 39, as described above.

When it is desired to acid treat an oil which is initially highly paraffinic, and required no extraction, this oil may be introduced into the process through a conduit 45 and valve 46, and the SO<sub>2</sub> soluble extract may be introduced into the oil from an outside source; it may be supplied by extracting an oil of low paraffinicity with 60 a selective solvent in the manner heretofore described, closing the valve 24, withdrawing the raffinate oil at 47, and utilizing the extract for admixture to the paraffinic oil which is supplied at 45.

65 To illustrate the process further, and to demonstrate the benefits to be derived from my process, the following example is given:

Example.—A Mid-Continent lubricating oil was extracted with furfural to produce a dark colored 70 raffinate oil having a viscosity index of 95 and a viscosity of 156 sec. Say. Univ. at 210° F. This raffinate could not be desludged by the ordinary methods of acid treatment, and would normally be clay treated. One portion of this raffinate 75

5 was contacted with 15% of activated clay at 450° F. Another portion was mixed with 6% of extract obtained by the above extraction, diluted with 50% naphtha, acid treated at 90° F. with 25 lbs. of 98% sulfuric acid per barrel of raffinate oil, settled to remove the sludge, and distilled to remove the naphtha. The remaining sour oil was contacted with 5% of activated clay at 450° F. The results of the two methods of treatment are given in the following table:

|                                                                            | Contacted with 15% activated clay | Acid treated and contacted with 5% activated clay |
|----------------------------------------------------------------------------|-----------------------------------|---------------------------------------------------|
| 15                                                                         |                                   |                                                   |
| Color, N. P. A.                                                            | 5+                                | 5+                                                |
| Visc., sec. Say. Univ. at 210° F.                                          | 151                               | 145                                               |
| Stability towards oxidation:<br>Visc. sec. Say. Univ. at 210° F.<br>after— |                                   |                                                   |
| 80 hrs.                                                                    | 175                               | 155                                               |
| 168 hrs.                                                                   | 230                               | 165                                               |
| 20                                                                         |                                   |                                                   |

\* Determined according to method outlined in National Petroleum News, 1933, vol. 25, No. 37, page 27 (Effect of Sludge on Engine Oil Performance, by Bernard, Rogers, Shoemaker and Wilkin).

25 From the above table it is apparent that acid  
treating in the manner previously described saves  
a considerable quantity of clay and improves the  
stability towards oxidation to a marked degree.  
Ordinarily, extraction solvents remove unsatu-  
30 rates and aromatics of the type soluble in liquid  
sulfur dioxide. Acid treating with sulfuric acid  
removes other unstable compounds insoluble in  
the selective solvents, or not sufficiently soluble  
therein to be effectively removed thereby, and  
35 consequently increases the stability of the oil.

My invention may be applied to oils of any viscosity, but is particularly effective to the more viscous oils, such as those having viscosities higher than 80 seconds Say. Univ. at 210° F., which are particularly difficult to treat with the known methods. I have found it preferable to employ an SO<sub>2</sub> soluble extract which has approximately the same viscosity as the oil being acid treated, so that the viscosity of the final product is not influenced by the viscosity of those portions of the added extract which are not removed with the acid sludge. Asphaltenes and asphaltic resins precipitated from oils containing them by means of light hydrocarbons such as propane, butane, naphtha, etc., or asphaltic materials obtained as distillation residues can also be used in addition to or in place of the above described SO<sub>2</sub> soluble extract.

**I claim as my invention:**

55 1. A process for refining lubricating oils, comprising the steps of extracting a lubricating oil containing paraffinic and non-paraffinic hydrocarbons with a selective solvent for non-paraffinic hydrocarbons under conditions causing the formation of a relatively small quantity of a first extract oil and a relatively large quantity of a first raffinate oil, further extracting the raffinate oil with a selective solvent of the same type to produce a second raffinate oil having a viscosity index greater than about 70, and a second extract oil, contacting the second raffinate oil with a concentrated strong mineral acid in the presence of at least a portion of the first extract oil, thereby forming an acid sludge, and separating the acid sludge from the sour oil.

60

65

70

2. The process according to claim 1 in which the first raffinate oil is mixed with an additional quantity of unextracted oil before being further extracted to produce the second raffinate oil.

75 3. In the process of refining a highly paraffinic

lubricating oil having a viscosity index greater than about 70, which upon treating with concentrated sulfuric acid produces pepper sludge not removable by settling, the improvement comprising adding to the said paraffinic oil a small quantity of a sulfur dioxide soluble mineral oil having approximately the same viscosity as the paraffinic oil, and treating the resulting mixture with concentrated sulfuric acid, thereby forming a sludge capable of settling.

4. The process according to claim 3 in which the initial oil has a viscosity of over 80 seconds Saybolt Universal at 210° F.

5. The process according to claim 3 in which the quantity of the extract is between 1 and 10% of the initial oil.

6. In the process of refining lubricating oils containing paraffinic and non-paraffinic hydrocarbons by solvent extraction to produce a paraffinic raffinate and a non-paraffinic extract oil, 20 said raffinate having a viscosity index greater than about 70 and producing upon treatment with concentrated sulfuric acid a pepper sludge not removable by settling, the improvement comprising returning a portion of the extract oil to 25 the said raffinate and treating the resulting mixture with concentrated sulfuric acid, thereby forming a sludge capable of settling.

7. A process for refining lubricating oils comprising the steps of extracting a lubricating oil fraction containing paraffinic and non-paraffinic hydrocarbons with a selective solvent for non-paraffinic hydrocarbons to produce a raffinate having a viscosity index greater than about 70 and an extract oil, further treating said extract oil to separate it into two fractions which, relative to each other, are more and less soluble in the selective solvent, and contacting the raffinate oil with concentrated sulfuric acid in the presence of at least a portion of the more soluble extract fraction, thereby producing an acid sludge, and separating the acid sludge from the sour oil. 30 35 40

8. In the process of refining a highly paraffinic lubricating oil having a viscosity index greater than about 70, which upon treating with concentrated sulfuric acid produces pepper sludge not removable by settling, the improvement comprising adding to the said paraffinic oil a sulfur dioxide-soluble mineral oil having approximately the same viscosity as the paraffinic oil in an amount insufficient materially to impair the viscosity index of the latter, and treating the resulting mixture with concentrated sulfuric acid, thereby forming a sludge capable of settling.

9. In the process of refining a highly paraffinic lubricating oil having a viscosity index greater than about 70, which upon treating with concentrated sulfuric acid produces pepper sludge not removable by settling, the improvement comprising adding to the said paraffinic oil a sulfur dioxide-soluble mineral lubricating oil in an amount insufficient materially to impair the viscosity index of the paraffinic lubricating oil, and treating the resulting mixture with concentrated sulfuric acid, thereby forming a sludge capable of settling. 55 60 65

10. In the process of refining a highly paraffinic lubricating oil having a viscosity index greater than about 70, which upon treating with concentrated sulfuric acid produces pepper sludge not removable by settling, the improvement comprising adding to the said paraffinic oil a sulfur dioxide-soluble mineral lubricating oil in an amount insufficient materially to impair the viscosity index of the paraffinic lubricating oil and 75

a small amount of a selective solvent for aromatic hydrocarbons, and treating the resulting mixture with concentrated sulfuric acid, thereby forming a sludge capable of settling.

5 11. The process of treating a petroleum oil which normally, upon treatment with sulfuric acid, gives rise to a peppery, not readily separable

sludge, with non-fuming sulfuric acid, which comprises agitating the oil with concentrated sulfuric acid in the presence of an added normally liquid unsaturated cyclic hydrocarbon in amount of from 1 to 10% of the oil, and separating the 5 sludge formed from the oil.

ALVIN P. ANDERSON.